

# UNITED STATES PATENT OFFICE.

HAROLD B. PULLAR, OF LAWRENCEVILLE, ILLINOIS.

## BITUMINOUS PRODUCT AND PROCESS OF MAKING THE SAME.

1,409,237.

Specification of Letters Patent. Patented Mar. 14, 1922.

No Drawing.

Application filed May 3, 1920. Serial No. 378,404.

*To all whom it may concern:*

Be it known that I, HAROLD B. PULLAR, a citizen of the United States, residing in the city of Lawrenceville, county of Lawrence, and State of Illinois, have invented certain new and useful Improvements in Bituminous Products and Processes of Making Same, of which the following is a specification.

My invention relates to an improvement in 10 bituminous products and relates more particularly to a product adaptable to numerous and varied uses such as a base for paint and varnish, as a special compound for producing high grade roofing cement; for waterproofing purposes, as a substitute for certain rubber products and innumerable other uses where a high grade bituminous product of a rubber-like and flexible nature is desirable.

20 Among its salient objects are to provide a special bituminous composition of a rubber like nature having a high melting point and one which is affected but little by extremes of temperature; to provide a cheap and improved substitute for stearine, cottonseed oil and other similar pitches which is more uniform in character, more constant in its consistency and is far less difficult to handle than those mentioned; to provide a process 30 for making this product and in general to provide a process and product of the character referred to.

Referring more particularly to the ingredients which are combined to make the product,—50% residuum oil and 50% cottonseed oil or stearine pitch are mixed and heated to a temperature of not less than 300° F., and not more than 400° F. This mixture is treated with air during the heating until 40 it attains a uniform quality and having a melting point or softening point of between 160° F. and 230° F., but from the disclosures herein made, the principles of my invention are capable of application to various other 45 improvements than those described, but in order to get a product of satisfactory quality for commercial use, it is necessary to adhere strictly to the above proportions, and it is also possible to produce and get the same 50 results by the addition of the proper amount of gilsonite or similar hard bitumen.

In the production of the bitumen compound as described in my invention it is possible to use any grade of cottonseed oil

or stearine pitch, and it is not essential that 55 these pitches be of uniform quality.

In order to obtain the best results the residuum oil is first placed in a kettle and heated to a temperature between 300° and 350° F. The pitch is then placed in a kettle 60 and allowed to slowly melt and mix with the oil. If the temperatures are raised over 350° F., there is apt to be a disintegration and separation and the results obtained as described in my invention cannot be pro- 65

After the pitch has been thoroughly melted and combines with the hot oil, air is forced through the pitch by means of air pipes at the bottom of the still for a period 70 varying from between 4 to 12 hours, depending upon the consistency of the product desired. Approximately between 1500 to 2000 cubic feet of air per minute should be forced through a batch of 18 tons, but this is not 75 essential as the time of completing a batch depends upon the quantity of air forced through it and temperature of the mixture.

I claim as my invention:

1. A product, comprising a mixture of a 80 vegetable pitch and oxidized residuum oil.

2. A mixture of stearine pitch and residuum oil oxidized with air and having added to it not more than 30% of a natural asphalt as gilsonite.

3. A product comprising in substantially 85 equal parts vegetable pitch and oxidized residuum oil, said product having a melting point between 160 and 230 degrees F.

4. An oxidized product consisting of non- 90 mineral pitchy material, oxidized residuum and gilsonite.

5. A product comprising a mixture of oxidized heavy oil and non-mineral pitch.

6. A mixture of a non-mineral pitch and 95 petroleum oil oxidized and having added to it natural asphalt.

7. A product comprising a mixture of oxidized residuum oil and non-mineral pitchy substance in approximately equal quantities, 100 said product having a melting point of not less than 160 degrees F.

8. A product comprising a mixture of non-mineral pitch, oxidized mineral oil and a natural asphalt, said product having a 105 melting point of not less than 160 degrees F.

HAROLD B. PULLAR.